

## UNITED STATES PATENT OFFICE.

WENDELL R. SWINT, OF WILMINGTON, DELAWARE, ASSIGNOR TO E. I. DU PONT DE NEMOURS & COMPANY, OF WILMINGTON, DELAWARE, A CORPORATION OF DELAWARE.

## HIGH-EXPLOSIVE COMPOSITION.

No Drawing.

Application filed April 13, 1922. Serial No. 552,345.

This invention relates to high explosives such as dynamite, and more particularly to nitroglycerine explosives of the permissible type.

5 The chief object of my invention is to provide explosive compositions of lower density than it has hitherto been feasible to manufacture.

10 Explosives of the permissible type have previously been made of such a density that a cartridge 1 1/4" in diameter and 8" long will weigh from 160-180 grams. An example of the composition of such an explosive is:

|                  | Per cent. |
|------------------|-----------|
| Nitroglycerine   | 10        |
| Ammonium nitrate | 80        |
| Wood flour       | 5         |
| Corn meal        | 5         |

20 Many variations have of course been made in formulas of this type, as for example, a substitution of from 3-20% sodium chloride for a corresponding proportion of ammonium nitrate; the use of similar percentages of sodium nitrate replacing ammonium nitrate; the substitution of other carbonaceous materials, such as starch, ivory nut meal, sawdust, wood pulp, etc., for corn meal or wood flour.

30 It is desirable for certain purposes to secure explosives of lower density than those at present available. The lowest density which it has hitherto been possible to obtain in explosives of this type corresponds to a weight of about 135 grams for a cartridge 1 1/4" in diameter and 8" long, and this is attained by the use of a specially high grade wood flour, which is expensive to manufacture.

45 I have discovered that bagasse pith, that is, the pith obtainable from sugar cane after extraction of the sugar therefrom, may be successively substituted for part or all of the carbonaceous, non-explosive, absorbent material commonly used in explosives of the kind above-mentioned, and that the resulting high explosive has a substantially lower density than corresponding explosives containing, as the absorbent ingredient, wood flour, 50 ivory nut meal, etc. Thus I have discovered that by substituting bagasse pith for wood flour and other carbonaceous materials, I can

produce explosives having a density corresponding to a weight of as low as 125 grams for a cartridge 1 1/4" in diameter and 8" long. In order to secure the desired results, the residue from sugar cane after the extraction of the sugar, and which is ordinarily in a crushed and macerated condition, may be screened to remove the greater percentage 55 of the long fibres, leaving only the pith. The bagasse pith as thus prepared may have a fiber content as high as 50%, but it is preferable that the amount be brought down to 25% or lower. Other methods of sugar manufacture in which the entire cane is first shredded and dried and then extracted with water to remove the sugar also may be utilized in obtaining bagasse pith of properties 60 which are satisfactory for use in my invention.

70 While my invention is capable of use in many different forms, for the purpose of illustration I will confine myself to the use of bagasse pith in explosives of the so-called permissible type which are used in coal mines where gas and dust exist in quantities which may be dangerous if ignited by the flame from an explosive.

75 As an example of my invention, I might use the following composition:

|                  | Per cent. |
|------------------|-----------|
| Nitroglycerine   | 10        |
| Ammonium nitrate | 75        |
| Sodium nitrate   | 5         |
| Bagasse pith     | 10        |

It should, however, be understood that I can vary such percentages quite widely and can introduce other ingredients without departing from the spirit of the invention. Thus, for example, I may use tetranitrodiglycerine in place of nitroglycerine in order to make the explosive low freezing, or I may omit sodium nitrate entirely or increase its percentage appreciably. Instead of sodium nitrate, I may use sodium chloride or I may use any of the well-known methods for depressing the temperature of the flame in order to secure an explosive which will be safe 100 to use in dusty and gaseous coal mines. For a portion of the bagasse pith, I may substitute other carbonaceous materials, such as corn meal, ivory nut meal, flour, etc.

The most important ranges of proportions of ingredients may be indicated as follows:

|                       | Per cent.  |
|-----------------------|------------|
| 5 Nitroglycerine----- | from 7-15  |
| Ammonium nitrate----- | from 40-85 |
| Sodium nitrate-----   | from 0-20  |
| Sodium chloride-----  | from 0-20  |
| Bagasse pith -----    | from 5-15  |

- 10 Although the most advantageous application of my invention is to the manufacture of permissible explosives, it is also useful, as above indicated, in the manufacture of other high explosives or dynamites. For example, 15 a typical dynamite, using bagasse as the chief absorbent ingredient, may have the following formula:

|                         | Parts. |
|-------------------------|--------|
| 20 Nitroglycerine ----- | 40     |
| Sodium nitrate-----     | 41     |
| Bagasse -----           | 8      |
| Sawdust-----            | 5      |
| Corn meal-----          | 5      |
| Chalk -----             | 1      |

I claim:

1. A non-gelatinized explosive composition containing a normally liquid high explosive, ammonium nitrate, and sufficient bagasse pith to substantially reduce the density of said composition.
2. An explosive composition of the permissible type comprising nitroglycerine, ammonium nitrate, a non-explosive salt adapted to reduce the flame temperature upon explosion of the composition, and sufficient bagasse pith to substantially reduce the density of said composition.
3. An explosive composition of the permissible type comprising ammonium nitrate, bagasse pith, sodium nitrate and from about 7 to 15% of nitroglycerine.
4. An explosive composition of the permissible type comprising nitroglycerine, ammonium nitrate, sodium nitrate, sodium chloride, and sufficient bagasse pith to substantially reduce the density of said composition.
5. An explosive composition characterized by its low density and comprising from about 7 to 15% of a normally liquid high explosive,

from about 5 to 15% of bagasse pith, and ammonium nitrate.

6. An explosive composition characterized by its low density and comprising from about 7 to 15% of a normally liquid high explosive, 55 from about 5 to 15% of bagasse pith, from 40 to 85% of ammonium nitrate, and a salt adapted to reduce the flame temperature upon explosion of the composition.

7. An explosive composition characterized by its low density and comprising from about 7 to 15% of nitroglycerine, from about 5 to 15% of bagasse pith, and ammonium nitrate.

8. An explosive composition having a 65 nitroglycerine content of about 12%, ammonium nitrate 40 to 85%, sodium nitrate about 5%, bagasse pith 5 to 15%, said explosive being of low density.

9. An explosive composition containing a 70 normally liquid high explosive, ammonium nitrate, and bagasse pith, the density of said composition being such that a cartridge thereof 1 1/4" in diameter and 8" long weighs about 125 grams.

10. An explosive composition of the permissible type comprising nitroglycerine, ammonium nitrate, a non-explosive salt adapted to reduce the flame temperature upon explosion of the composition, and sufficient bagasse pith to reduce the density of said composition to a value such that a cartridge thereof 1 1/4" in diameter and 8" long weighs substantially less than 135 grams.

11. An explosive composition comprising 85 from about 7 to 15 per cent of a normally liquid high explosive, from about 5 to 15 per cent of bagasse pith, and ammonium nitrate, the density of said composition being such that a cartridge thereof 1 1/4" in diameter and 8" long weighs substantially less than 135 grams.

12. An explosive composition comprising from about 7 to 15 per cent of a normally liquid high explosive, from about 5 to 15 per cent of bagasse pith, and ammonium nitrate, the density of said composition being such that a cartridge thereof 1 1/4" in diameter and 8" long weighs about 125 grams.

In testimony whereof I affix my signature.

WENDELL R. SWINT.